# EUROPEAN PATENT SPECIFICATION

(11) **EP 2 278 416 B1**
(45) Date of publication and mention of the grant of the patent: **11.09.2013**
(21) Application number: 10169814.0
(22) Date of filing: 16.07.2010
(51) Int. Cl.: G03G 15/20, G03G 15/00

(54) **Fuser component**
Fixierelement
Elément de fixage

(30) Priority: 24.07.2009 US 509393
(43) Date of publication of application: 26.01.2011
(73) Proprietor: Xerox Corporation, Rochester, New York 14644 (US)
(72) Inventor: Gilmartin, Brian P., Williamsville, NY 14221 (US); Lin, Liang-Bih, Rochester, NY 14618 (US)
(74) Representative: Grünecker, Kinkeldey, Stockmair & Schwanhäusser

(56) References cited:
- EP-A2- 0 454 030
- US-A- 5 208 318
- US-A- 5 248 339

## Description

### BACKGROUND

The presently disclosed invention relates generally to a fuser component comprising a cross-linked protective outer coating or layer that withstands high temperatures and which maintains integrity in such conditions. More particularly, the present embodiments pertain to a fuser component having an outer coating comprised of a cross-linking composition that improves resistance to thermal degradation and extends the service life of the fuser component.

There is provided a fuser member comprising a protective outer coating or layer. In embodiments, the outer layer is positioned on a substrate, which may be of many configurations including a roller, belt, film, or substrate. In other embodiments, the outer layer has an outer release layer thereon. In further embodiments, there is positioned between the substrate and the outer layer, an intermediate and/or adhesive layer. The present invention may be useful as fuser members in xerographic machines, including color machines.

In a typical electrostatographic reproducing apparatus, a light image of an original to be copied is recorded in the form of an electrostatic latent image upon a photosensitive member and the latent image is subsequently rendered visible by the application of electroscopic thermoplastic resin particles which are commonly referred to as toner. The visible toner image is then in a loose powdered form and can be easily disturbed or destroyed. The toner image is usually fixed or fused upon a support, which may be the photosensitive member itself, or other support sheet such as plain paper.

The use of thermal energy for fixing toner images onto a support member is well known and methods include providing the application of heat and pressure substantially concurrently by various means, a roll pair maintained in pressure contact, a belt member in pressure contact with a roll, a belt member in pressure contact with a heater. Heat may be applied by heating one or both of the rolls, plate members, or belt members. With a fixing apparatus using a thin film in pressure contact with a heater, the electric power consumption is small, and the warming-up period is significantly reduced or eliminated.

It is important in the fusing process that the materials used or incorporated into the fuser components can withstand high temperatures and are resistant to thermal degradation as such components operate in and/or generate high heat.

Known fuser coatings include high temperature polymers such as polytetrafluoroethylene, perfluoroalkoxy, fluorinated ethylene propylene, silicone rubber, and fluorosilicone rubber, and fluoroelastomers. However, these coatings do not tend to stay clean during use. Further, the coatings often wear during use and/or become scratched during operation. In addition, these known surfaces often react with the toner, oil or debris from media, which causes the surface to become dirty and/or contaminated. The surface can, in turn, become physically damaged and results in a fuser member having a reduced useful function and short life.

Therefore, a need remains for fuser components for use in electrostatographic machines that have superior mechanical properties, including high resistance to thermal degradation. In addition, a need remains for prolonging fuser component service life despite the harsh operating conditions.

EP-A-0454030 discloses an electrostratographic toner fusing member having a support and a layer comprising a crosslinked fluoroelastomer, characterized in that the fluoroelastomer is a crosslinked polyfluorophosphazene elastomer.

US Patent 5,208,318 relates to specific phosphazene-containing amines used as curing agents for the polymerization of phthalonitrile monomers and oligomeric resins and a method therefor.

### SUMMARY

According to aspects illustrated herein, there is provided a fuser component comprising a substrate, and an outer layer disposed on the substrate, wherein the outer layer comprises a phosphonitrilic trimer as defined in claim 1.

Yet another embodiment, there is provided an image forming apparatus for forming images on a recording medium comprising a charge-retentive surface to receive an electrostatic latent image thereon, a development component to apply toner to said charge-retentive surface to develop an electrostatic latent image to form a developed image on said charge retentive surface, a transfer film component to transfer the developed image from said charge retentive surface to a copy substrate, and a fusing component for fusing toner images to a surface of said copy substrate, said fusing component comprising a substrate, and an outer layer disposed on the substrate, wherein the outer layer is formed from a solution as defined in claim 13.

Preferred embodiments are set forth in the subclaims.

### BRIEF DESCRIPTION OF THE DRAWINGS

For a better understanding, reference may be made to the accompanying figures.

FIG. 1 is an illustration of a general electrostatographic apparatus;

FIG. 2 is a sectional view of a fusing belt and pressure roller in accordance with the present embodiments;

FIG. 3 is a sectional view of a pressure belt and fuser roller in accordance with the present embodiments;

FIG. 4 is a schematic illustration of a fuser component having a two-layer configuration in accordance with the present embodiments; and

FIG. 5 is a graph illustrating high resistance to thermal degradation exhibited by an outer coating in accordance with the present embodiments.

### DETAILED DESCRIPTION

In the following description, reference is made to the accompanying drawings, which form a part hereof and which illustrate several embodiments

The presently disclosed embodiments are directed to fuser component comprising a protective outer layer comprising a novel composition that facilitates a high degree of cross-linking such that the resulting outer layer is highly resistant to thermal degradation. The outer coating comprises a phosphonitrilic trimer and film-forming resin which cross-link in the presence of an acid catalyst to form a coating that is able to remain intact in temperatures that known coating compositions could not. Such fuser members exhibit improved wear resistance and life extension.

Inorganic polymers comprised of phosphonitrilic compounds have been studied as alternatives to organic polymers. Phosphonitrilic polymers offer a relatively simplistic means of achieving structure-function relationship, which generates a broader range of physical properties compared to organic materials. Phosphonitrilic polymers have desirable properties (e.g., thermal resistance, electrical properties, hydrophobicity/hydrophilicity, biomedical applications) which can be tailored through syntheses based on the side chain groups of the respective monomer(s).

The present embodiments are based upon cross-linking a new phosphonitrilic trimer with a film-forming resin to form a protective coating. The phosphonitrilic trimer has six alkoxyalkyl linkages and, in the presence of an acid catalyst, is able to cross-link with the resin to form a coating that is highly resistant to thermal degradation. In particular embodiments, the acid catalyst is selected from the group consisting of p-toluenesulfonic acid, dinonylnaphthalenesulfonic acid, dinonylnaphthalenedisulfonic acid, dodecylbenzenesulfonic acid, and mixtures thereof. The new coating of the present embodiments demonstrate complete improved thermal stability (e.g., complete decomposition at temperatures of greater than 800 °C by thermogravimetric analysis), substantially higher than typically seen from organic resins such as melamine and polyol which generally degrade at about 600 °C. In addition, the coating exhibits excellent resistance against concentrated acids and is also harder than several commercially available polymers, such as high and low density polyethylene and polystyrene.

As discussed above, the phosphonitrilic trimer prepared with six alkoxyalkyl groups. It has structural features that are similar to commercially available melamines (such as hexamethoxymethylmelamine, Cymel 303 available from Cytec Industries Inc. (West Paterson, New Jersey)), but with twice the potential cross-linking amino groups. In the presence of an acid catalyst, the phosphonitrilic trimer cross-links with a film-forming resin. This is similar to the reaction that some melamines have in which the melamines cross-link, in the presence of an acid catalyst, with hydroxyl-, carboxyl-, and/or amide containing compounds through alkoxy linkages. The phosphonitrilic trimer has the following structure: wherein Rᵢ and Rᵢᵢ are independently selected alkyl groups or derivatives thereof.

In embodiments, the the phosphonitrilic trimer has a molecular weight (Mw) of from 300 to 900 g/mol, or from 500 to 700 g/mol. The phosphonitrilic trimer compound may be in gelatinous form and is miscible in organic solvents.

In further embodiments, the phosphonitrilic trimer is present in the outer coating or layer in an amount of from 5 percent to 95 percent, or from 50 percent to 75 percent by weight of the total weight of the outer coating or layer. In other embodiments, the film-forming resin is present in the outer coating or layer in an amount of from 5 percent to 95 percent, or from 25 percent to 50 percent by weight of the total weight of the outer coating or layer. In embodiments, a ratio of the phosphonitrilic trimer to the resin in the outer layer is from 0.5 to 3. In embodiments, the film-forming resin can be selected from, but are not limited to, thermoplastic and thermosetting resins such as polycarbonates, polyesters, polyurethanes, polystyrenes, polyarylethers, polyarylsulfones, polysulfones, polyethersulfones, polyphenylene sulfides, polyvinyl acetate, polyacrylates, polyvinyl acetals, polyamides, polyimides, amino resins, phenolic resins, phenoxy resins, epoxy resins, phenylene oxide resins, polystyrene and acrylonitrile copolymers, vinyl acetate copolymers, acrylate copolymers, alkyd resins, styrene-butadiene copolymers, styrene-alkyd resins, polyvinylcarbazole, and mixtures thereof. In particular embodiments, the resin may be selected from the group consisting of acrylic polyol, polyether polyol, polyester polyol, and mixtures thereof. In further embodiments, the protective outer coating or layer has a thickness of from 0.1 to 50 µm, or from 5 to 40 µm.

The exemplary embodiments of this disclosure are described below with reference to the drawings. The same reference numerals are used to identify the same structure in different figures unless specified otherwise. In addition, though the discussion will address negatively charged systems, the imaging members of the present disclosure may also be used in positively charged systems. The present invention is directed to fuser components, and in particular, fusing components including fuser members, pressure members, donor members, external heat members, and other components that operate in and/or generate high temperatures. In embodiments, the fuser member can be a pressure belt, fuser roller, fusing belt, and pressure roller.

The fuser component comprises a substrate and a protective outer layer comprising a phosphonitrilic timer cross-linked with a film-forming resin. In other embodiments, the fuser component comprises a substrate having the protective outer layer and an outer release layer disposed on the protective outer layer. In yet other embodiments, optional adhesive and/or intermediate layers can be present between the substrate and the protective outer layer, and/or between the protective outer layer and the outer release layer.

Referring to FIG. 1, in a typical electrostatographic reproducing apparatus, a light image of an original to be copied is recorded in the form of an electrostatic latent image upon a photosensitive member and the latent image is subsequently rendered visible by the application of electroscopic thermoplastic resin particles which are commonly referred to as toner. Specifically, photoreceptor 10 is charged on its surface by means of a charger 12 to which a voltage has been supplied from power supply 11. The photoreceptor is then imagewise exposed to light from an optical system or an image input apparatus 13, such as a laser and light emitting diode, to form an electrostatic latent image thereon. Generally, the electrostatic latent image is developed by bringing a developer mixture from developer station 14 into contact therewith.

Development can be effected by use of a magnetic brush, powder cloud, or other known development process. A dry developer mixture usually comprises carrier granules having toner particles adhering triboelectrically thereto. Toner particles are attracted from the carrier granules to the latent image forming a toner powder image thereon. Alternatively, a liquid developer material may be employed, which includes a liquid carrier having toner particles dispersed therein. The liquid developer material is advanced into contact with the electrostatic latent image and the toner particles are deposited thereon in image configuration.

After the toner particles have been deposited on the photoconductive surface, in image configuration, they are transferred to a copy sheet 16 by transfer means 15, which can be pressure transfer or electrostatic transfer. Alternatively, the developed image can be transferred to an intermediate transfer member and subsequently transferred to a copy sheet.

After the transfer of the developed image is completed, copy sheet 16 advances to fusing station 19, depicted in FIG. 1 as fusing and pressure rolls, wherein the developed image is fused to copy sheet 16 by passing copy sheet 16 between the fusing and pressure members, thereby forming a permanent image. Photoreceptor 10, subsequent to transfer, advances to cleaning station 17, wherein any toner left on photoreceptor 10 is cleaned therefrom by use of a blade, brush, or other cleaning apparatus.

FIG. 2 shows a sectional view of an example of a fusing apparatus 19 according to an embodiment of the present invention. In FIG. 2, a heat resistive film or an image fixing film 24 in the form of an endless belt is trained or contained around three parallel members, that is, a driving roller 25, a follower roller 26 of metal and a low thermal capacity linear heater 20 disposed between the driving roller 25 and the follower roller 26. The follower roller 26 also functions as a tension roller for the fusing belt 24. The fusing belt rotates at a predetermined peripheral speed in the clockwise direction by the clockwise rotation of the driving roller 25. The peripheral speed is the same as the conveying speed of the sheet having an image thereon so that the film is not creased, skewed or delayed.

A pressure roller 28 has a rubber elastic layer with parting properties, such as silicone rubber or the like, and is press-contacted to the heater 20 with the bottom travel of the fusing belt 24 therebetween. The pressure roller is pressed against the heater at the total pressure of 4-7 kg by an urging means (not shown). The pressure roller rotates co-directionally, that is, in the counterclockwise direction, with the fusing belt 24. In the present embodiments, the protective outer layer can be coated on the fuser belt and/or on the pressure roller.

The heater 20 is in the form of a low thermal capacity linear heater extending in a direction crossing with the film 24 surface movement direction (film width direction). It comprises a heater base 27 having a high thermal conductivity, a heat generating resistor 22 generating heat upon electric power supply thereto, and a temperature sensor 23, and is mounted on a heater support 21 having high thermal conductivity.

The heater support 21 supports the heater 20 with thermal insulation on an image fixing apparatus and is made from high heat durability resin such as PPS (polyphenylene sulfide), PAI (polyamideimide), PI (polyimide), polyaramide, polyphthalamide, polyketones, PEEK (polyether ether ketone) or liquid crystal polymer material, or a compound material of such resin material and ceramics, metal, or glass.

An example of the heater base 27 is in the form of an alumina plate having a thickness of 1.0 mm, a width of 10 mm and a length of 240 mm comprised of a high conductivity ceramic material.

The heat generating resistor material 22 is applied by screen printing or the like along a longitudinal line substantially at the center, of the bottom surface of the base 27. The heat generating material 22 is, for example, Ag/Pd (silver palladium), Ta2N or another electric resistor material having a thickness of approximately 10 microns and a width of 1-3 mm. It is coated with a heat resistive glass 21 a in the thickness of approximately 10 microns, as a surface protective layer. A temperature sensor 23 is applied by screen printing or the like substantially at a center of a top surface of the base 27 (the side opposite from the side having the heat generating material 22). The sensor is made of Pt film having low thermal capacity. Another example of the temperature sensor is a low thermal capacity thermistor contacted to the base 27.

The linear or strip heater 22 is connected with the power source at the longitudinal opposite ends, so that the heat is generated uniformly along the heater. The power source in this example provides AC 100 V, and the phase angle of the supplied electric power is controlled by a control circuit (not shown) in accordance with the temperature detected by the temperature detecting element 23.

A film position sensor 42 in the form of a photocoupler is disposed adjacent to a lateral end of the film 24. In response to the output of the sensor, the roller 26 is displaced by a driving means in the form of a solenoid (not shown), so as to maintain the film position within a predetermined lateral range.

Upon an image formation start signal, an unfixed toner image is formed on a recording material at the image forming station. The copy sheet 16 having an unfixed toner image Ta thereon is guided by a guide 29 to enter between the fusing belt 24 and the pressure roller 28 at the nip N (fixing nip) provided by the heater 20 and the pressure roller 28. Copy sheet 16 passes through the nip between the heater 20 and the pressure roller 28 together with the fusing belt 24 without surface deviation, crease or lateral shifting while the toner image carrying surface is in contact with the bottom surface with the fusing belt 24 moving at the same speed as copy sheet 16.

The heater 20 is supplied with electric power at a predetermined timing after generation of the image formation start signal so that the toner image is heated at the nip so as to be softened and fused into a softened or fused image Tb.

Fusing belt 24 is sharply bent at an angle theta of, for example, about 45 degrees at an edge S (the radius of curvature is approximately 2 mm), that is, the edge having a large curvature in the heater support 21. Therefore, the sheet advanced together with the film 24 in the nip is separated by the curvature from the fusing belt 24 at edge S. Copy sheet 16 is then discharged to the sheet discharging tray. By the time copy sheet 16 is discharged, the toner has sufficiently cooled and solidified and therefore is completely fixed (toner image Tc).

In this embodiment, heat generating element 22 and base 27 of heater 20 have low thermal capacity. In addition, heater element 22 is supported on support 21 through thermal insulation. The surface temperature of heater 20 in the nip quickly reaches a sufficiently high temperature, which is necessary in order to fuser, the toner. Also, a stand-by temperature control is used to increase the temperature of the heater 20 to a predetermined level. Therefore, power consumption can be reduced, and rise in temperature can be prevented.

The fusing belt is in contact with the heater. The distance between the outer layer of the fusing belt and the heater is preferably from 0.5 mm to 5.0 mm. Similarly, the distance between the fusing belt and the grounded rollers 25 and 26 is not less than 5 mm and is, for example, from 5 to 25 mm. These distances prevent leakage of the charge applied to the copy sheet 16 by an image (not shown) forming station from leaking to the ground through the copy sheet 16. Therefore, possible deterioration of image quality due to improper image transfer can be avoided, or minimized.

In another embodiment of the invention, the fusing belt may be in the form of a sheet. For example, a non-endless film may be rolled on a supply shaft and taken out to be wrapped on a take-up shaft through the nip between the heater and the pressure roller. Thus, the film may be fed from the supply shaft to the take-up shaft at the speed, which is equal to the speed of the transfer material, reference U.S. Patent No. 5,157,446.

Another embodiment is depicted in FIG. 3, wherein the fuser member is in the form of a fuser roller 37 having internal heater 38 positioned inside the fuser member. In an optional embodiment, the heating member 38 can be positioned on the outside of the fusing member. Pressure belt 39 cycles around rollers 25, 26, and 40. In this alternative configuration, the toner or other marking material is fused to the copy substrate 16 by fuser roller 37. The load on pad 41 is approximately 1.7 kgf. In embodiments, the protective outer layer can be coated on the fuser roller and/or on the pressure belt.

The fusing component of the present invention can be comprised of various different configurations. In one embodiment of the invention, the fusing component 50 is of a two-layer configuration as shown in FIG. 4. It is understood that this and other configurations herein, can be used on any fusing component that operates in and/or generates high heat. In this embodiment, the fusing component 50 comprises substrate 52 having optional fillers 54 dispersed or contained therein. Positioned over the substrate is the protective outer layer 56 having the phosphonitrilic trimer 60 cross-linked or contained therein. The embodiments also provide for a three layer configuration in which an outer release layer may be positioned over the protective outer layer or that an adhesive or other intermediate layer or layers may be present between the substrate and the protective outer layer.

Examples of suitable substrate materials include in the case of roller or film-type substrates, metals such as aluminum, stainless steel, steel, and nickel. In the case of film-type substrates, suitable substrates include high temperature plastics that are suitable for allowing a high operating temperature (i.e., greater than about 80 °C, preferably greater than 200 °C), and capable of exhibiting high mechanical strength. In embodiments, the plastic has a flexural strength of from 2,000,000 to 3,000,000 psi, and a flexural modulus of from 25,000 to 55,000 psi.

Plastics possessing the above characteristics and which are suitable for use as the substrate for the fuser members include epoxy; polyphenylene sulfide such as that sold under the tradenames FORTRON available from Hoechst Celanese, RYTON R-4 available from Phillips Petroleum, and SUPEC available from General Electric; polyimides such as polyamideimide sold under the tradename TORLON 7130 available from Amoco; polyketones such as those sold under the tradename KADEL E1230 available from Amoco, polyether ether ketone sold under the tradename PEEK 450GL30 from Victrex, polyaryletherketone; polyamides such as polyphthalamide sold under the tradename AMODEL available from Amoco; polyethers such as polyethersulfone, polyetherimide, polyaryletherketone; polyparabanic acid; liquid crystalline resin (XYDAR) available from Amoco; ULTEM available from General Electric; ULTRAPEK available from BASF; and mixtures thereof. Other suitable substrate materials include fluoroelastomers such as those sold under the tradename VITON from DuPont; silicone rubbers, and other elastomeric materials. The substrate may also comprise a mixture of any of the above materials.

The substrate as a film, sheet, or belt, has a thickness of from 25 to 250, or from 60 to 100 micrometers.

The protective outer layer material is suitable for allowing a high operating temperature. For example, in embodiments the protective outer layer material can operate in a temperature greater than 80 °C, or greater than 200 °C. In more specific embodiments, the protective outer layer material can operate in a temperature from 150 °C to 400 °C, or from 200 °C to 350 °C. As a result, the fuser components having an outer layer or coating of the protective material are capable of exhibiting high mechanical strength and optionally possessing tailored electrical properties.

The fusing component employed for the present invention can be of any suitable configuration. Examples of suitable configurations include a sheet, a film, a web, a foil, a strip, a coil, a cylinder, a drum, a roller, an endless strip, a circular disc, a belt including an endless belt, an endless seamed flexible belt, and an endless seamless flexible belt, an endless belt having a puzzle cut seam.

Optionally, any known and available suitable adhesive layer may be positioned between the protective outer layer and the substrate, and/or between the protective outer layer and the outer release layer. Examples of suitable adhesives include silanes such as amino silanes (such as, for example, A1100 from OSI Specialties, Friendly West Virginia), titanates, zirconates, aluminates, and mixtures thereof. In an embodiment, an adhesive in from 0.25 to 10 percent solution, can be wiped on the substrate. The adhesive layer can be coated on the substrate, or on the polyimide outer layer, to a thickness of from 2 to 2,000 nanometers, or from 2 to 500 nanometers. The adhesive can be coated by any suitable, known technique, including spray coating or wiping.

Various exemplary embodiments encompassed herein include a method of imaging which includes generating an electrostatic latent image on an imaging member, developing a latent image, and transferring the developed electrostatic image to a suitable substrate.

While the description above refers to particular embodiments, it will be understood that many modifications may be made.

The presently disclosed embodiments are, therefore, to be considered in all respects as illustrative and not restrictive, the scope of embodiments being defined by the appended claims rather than the foregoing description.

### EXAMPLES

The example set forth herein below and is illustrative of different compositions and conditions that can be used in practicing the present embodiments.

Example 1

Preparation of the Phosphonitrilic Trimer:

Hexakis(methoxyethylamino)tricyclophosphene (HMEAT) was prepared by adding 10.04 g (28.9 mmol) of phosphonitrilic chloride trimer, along with 200 mL of toluene and 100 mL of triethylamine into a 1 L round bottom flask. The solution was stirred until all solids had dissolved, at which point 26.01 g (346 mmol) of 2-methoxyethylamine was added slowly. This produced a white precipitate almost immediately in the solution. The sample was allowed to reflux for 4 days. The solution was then cooled to room temperature and the solid was filtered off and washed with toluene. The organics were combined and evaporated of solvent and excess base under reduced pressure, leaving the product (13.61 g; 81.3% yield) as a yellow gel. ¹H (500 MHz, THF-d₈) δ 3.45 (t, 2H), 3.33 (s, 3H), 3.05 (br s, 2H). ³¹P (200 MHz, CD₂Cl₂) δ 18.15. The reaction is shown as follows: The cross-linking properties of the molecule were investigated by preparing a formulation composed of HMEAT and a resin. The solution for film preparation comprised a 60:40 mixture (by weight) of HMEAT and JONCRYL 587 polyol (available from BASF Corp. (Florham Park, New Jersey)) in 1-methoxy-2-propanol (DOWANOL PM, available from The Dow Chemical Co. (Midland, Michigan)). NACURE XP-357 acid catalyst (available from King Industries, Inc. (Norwalk, Connecticut)) was also added to accelerate the cross-linking (1.0 wt% total solids). The solution was coated on a glass plate using a 5 mil bird bar and dried in a convection oven at 185 °C for 1 hour and resulting in about 30 µm film.

The average hardness of the cured film, analyzed using a nanoindenter, was determined to be 40 ± 2 MPa, which is harder than some commercially available plastics (see Table 1). In addition, the film demonstrated no degradation in the presence of concentrated hydrochloric acid (12.1 N). In fact, concentrated nitric acid (15.8 N) was required to remove the film from the glass substrate.

**Table 1**

| POLYMER | AVERAGE HARDNESS (MPa) |
|---|---|
| 60:40 HMEAT/JONCRYL 587 | 40 |
| HD Polyethylene | 32 |
| LD Polyethylene | 10 |
| Polystyrene | 34 |
| Ethylene Vinyl Acetate | 10-20 |

The thermal stability of a film prepared from the mixture above was compared to that from a mixture of 60:40 CYMEL 303/JONCRYL 587 by thermogravimetric analysis (TGA). As shown in FIG. 5, analysis showed that both samples began to degrade after 200 °C. However, at 600 °C almost all of the CYMEL 303/JONCRYL 587 film (bottom two lines represented by square and x) had decomposed, while nearly 40% of the HMEAT/JONCRYL 587 film (top two lines represented by diamond and triangle) remained intact. In fact, a small amount of the HMEAT/JONCRYL 587 film is still present at 800 °C.

FIG. 5 shows thermogravimetric analysis plots of 60:40 CYMEL 303/JONCRYL 587 as compared to HMEAT/JONCRYL 587. As can be seen, the inventive film exhibited much higher resistance to thermal degradation than the control sample.

In summary, the inventors of the present disclosure have prepared a novel phosphonitrilic trimer which has six alkoxyalkyl groups that facilitate cross-linking with a film-forming resin in the presence of an acid catalyst to form a protective coating. The inventive coating shows greater thermal stability than a formulation composed of a commercially available organic melamine and polyol. In addition, the present embodiments provide a film that is resistant to concentrated hydrochloric acid and has an average hardness greater than commonly known polymers.

## Claims

1. A fuser component comprising:
a substrate; and
an outer layer disposed on the substrate, wherein the outer layer comprises a phosphonitrilic trimer, wherein said outer layer is formed from a solution comprising a phosphonitrilic trimer, resin and an acid catalyst in a solvent,
wherein the phosphonitrilic trimer has the structure:
wherein Rᵢ and Rᵢᵢ are independently selected alkyl groups or derivatives thereof, and
wherein the phosphonitrilic trimer is crosslinked with the resin.

2. The component of claim 1, wherein the resin comprises thermoplastic and thermosetting resins selected from the group consisting of polycarbonates, polyesters, polyurethanes, polystyrenes, polyarylethers, polyarylsulfones, polysulfones, polyethersulfones, polyphenylene sulfides, polyvinyl acetate, polyacrylates, polyvinyl acetals, polyamides, polyimides, amino resins, phenolic resins, phenoxy resins, epoxy resins, phenylene oxide resins, polystyrene and acrylonitrile copolymers, vinyl acetate copolymers, acrylate copolymers, alkyd resins, styrenebutadiene copolymers, styrene-alkyd resins, polyvinyl carbazole, and mixtures thereof, optionally wherein the resin is selected from the group consisting of acrylic polyol, polyether polyol, polyester polyol, and mixtures thereof.

3. The component of claim 1, wherein the acid catalyst is selected from the group consisting of p-toluenesulfonic acid, dinonylnaphthalenesulfonic acid, inonylnaphthalenedisulfonic acid, dodecylbenzenesulfonic acid, and mixtures thereof.

4. The component of claim 1, wherein the substrate comprises a material selected from the group consisting of metals and polymers.

5. The component of claim 1, wherein the phosphonitrilic trimer is present in an amount of from 5 percent to 95 percent by weight of the total weight of the outer layer, optionally
wherein the phosphonitrilic trimer is present in an amount of from 50 percent to 75 percent by weight of the total weight of the outer layer.

6. The component of claim 1, wherein the resin is present in an amount of from 5 percent to 95 percent by weight of the total weight of the outer layer.

7. The component of claim 1, wherein the phosphonitrilic trimer has a molecular weight (Mw) of from 300 to 900, or
wherein the outer layer has a thickness from 0.1 to 50 µm.

8. The component of claim 1 being a xerographic component, optionally
wherein the xerographic component is selected from the group consisting of fuser component and photoreceptor component.

9. The component of claim 8, wherein the fuser component is selected from a pressure component, a fuser component, a donor component, and a heating component.

10. The component of claim 1, wherein a ratio of the phosphonitrilic trimer to the resin is from 0.5 to 3.

11. The component of claim 1, wherein the component has a substantially higher resistance to thermal degradation as compared to a component without the outer layer.

12. A fuser component according to claim 1 wherein the fuser component is selected from the group consisting of a pressure belt, fuser roller, fusing belt, and pressure roller, optionally further including other layers selected from the group consisting of an outer release layer, an intermediate layer and an adhesive layer.

13. An image forming apparatus for forming images on a recording medium comprising:
a charge-retentive surface to receive an electrostatic latent image thereon;
a development component to apply toner to said charge-retentive surface to develop an electrostatic latent image to form a developed image on said charge retentive surface;
a transfer film component to transfer the developed image from said charge retentive surface to a copy substrate; and
a fusing component for fusing toner images to a surface of said copy substrate, said fusing component comprising
a substrate, and
an outer layer disposed on the substrate, wherein said outer layer is formed from a solution comprising a phosphonitrilic trimer, resin and an acid catalyst in a solvent,
wherein the phosphonitrilic trimer has the structure:
wherein Rᵢ and Rᵢᵢ are independently selected alkyl groups or derivatives thereof, and
wherein the phosphonitrilic trimer is crosslinked with the resin.

## Patentansprüche

1. Schmelzfixierkomponente umfassend:
ein Substrat; und
eine auf dem Substrat angeordnete äußere Schicht, wobei die äußere Schicht ein Phosphonitriltrimer umfasst, wobei die äußere Schicht aus einer Lösung gebildet ist, die ein Phosphonitriltrimer, Harz und einen Säurekatalysator in einem Lösungsmittel umfasst,
wobei das Phosphonitriltrimer die Struktur aufweist:
wobei Rᵢ und Rᵢᵢ unabhängig voneinander ausgewählte Alkylgruppen oder Derivate davon sind und wobei das Phosphonitriltrimer mit dem Harz vernetzt ist.

2. Komponente nach Anspruch 1, wobei das Harz thermoplastische und wärmehärtbare Harze umfasst, die ausgewählt sind aus der Gruppe bestehend aus Polycarbonaten, Polyestern, Polyurethanen, Polystyrolen, Polyarylethern, Polyarylsulfonen, Polysulfonen, Polyethersulfonen, Polyphenylensulfiden, Polyvinylacetat, Polyacrylaten, Polyvinylacetalen, Polyamiden, Polyimiden, Aminoharzen, Phenolharzen, Phenoxyharzen, Epoxyharzen, Phenylenoxidharzen, Polystyrol- und Acrylnitril-Copolymeren, Vinylacetat-Copolymeren, Acrylat-Copolymeren, Alkydharzen, Styrol-Butadien-Copolymeren, Styrol-Alkydharzen, Polyvinylcarbazol und Mischungen davon, wobei das Harz gegebenenfalls ausgewählt ist aus der Gruppe bestehend aus Acrylpolyol, Polyetherpolyol, Polyesterpolyol und Mischungen davon.

3. Komponente nach Anspruch 1, wobei der Säurekatalysator ausgewählt ist aus der Gruppe bestehend aus p-Toluolsulfonsäure, Dinonylnaphthalinsulfonsäure, Dinonylnaphthalindisulfonsäure, Dodecylbenzolsulfonsäure und Mischungen davon.

4. Komponente nach Anspruch 1, wobei das Substrat ein Material umfasst, das ausgewählt ist aus der Gruppe bestehend aus Metallen und Polymeren.

5. Komponente nach Anspruch 1, wobei das Phosphonitriltrimer in einer Menge von 5 bis 95 Gew.-%, bezogen auf das Gesamtgewicht der äußeren Schicht, vorhanden ist, wobei das Phosphonitriltrimer gegebenenfalls in einer Menge von 50 bis 75 Gew.-%, bezogen auf das Gesamtgewicht der äußeren Schicht, vorhanden ist.

6. Komponente nach Anspruch 1, wobei das Harz in einer Menge von 5 bis 95 Gew.-%, bezogen auf das Gesamtgewicht der äußeren Schicht, vorhanden ist.

7. Komponente nach Anspruch 1, wobei das Phosphonitriltrimer ein Molekulargewicht (Mw) von 300 bis 900 aufweist, oder
wobei die äußere Schicht eine Dicke von 0,1 bis 50 µm aufweist.

8. Komponente nach Anspruch 1, bei der es sich um eine xerographische Komponente handelt,
wobei die xerographische Komponente gegebenenfalls ausgewählt ist aus der Gruppe bestehend aus einer Schmelzfixierkomponente und einer Photorezeptorkomponente.

9. Komponente nach Anspruch 8, wobei die Schmelzfixierkomponente ausgewählt ist aus einer Druckkomponente, einer Schmelzfixierkomponente, einer Donorkomponente und einer Heizkomponente.

10. Komponente nach Anspruch 1, wobei ein Verhältnis des Phosphonitriltrimers zu dem Harz 0,5 bis 3 beträgt.

11. Komponente nach Anspruch 1, wobei die Komponente eine wesentlich höhere Beständigkeit gegenüber einem thermischen Abbau im Vergleich zu einer Komponente ohne die äußere Schicht aufweist.

12. Schmelzfixierkomponente nach Anspruch 1, wobei die Schmelzfixierkomponente ausgewählt ist aus der Gruppe bestehend aus einem Druckband, einer Schmelzfixierwalze, einem Schmelzfixierband und einer Druckwalze, gegebenenfalls außerdem weitere Schichten enthaltend, die ausgewählt sind aus der Gruppe bestehend aus einer äußeren Trennschicht, einer Zwischenschicht und einer Klebschicht.

13. Bilderzeugende Apparatur zum Erzeugen von Bildern auf einem Aufzeichnungsmedium umfassend:
eine ladungszurückhaltende Oberfläche zum Aufnehmen eines elektrostatischen Latentbilds darauf;
eine Entwicklungskomponente zum Aufbringen von Toner auf die ladungszurückhaltende Oberfläche, um ein elektrostatisches Latentbild zu entwickeln, um ein entwickeltes Bild auf der ladungszurückhaltenden Oberfläche zu bilden;
eine Übertragungsfilmkomponente zum Übertragen des entwickelten Bildes von der ladungszurückhaltenden Oberfläche auf ein Kopiesubstrat; und
eine Schmelzfixierkomponente zum Schmelzfixieren von Tonerbildern auf eine Oberfläche des Kopiesubstrats, wobei die Schmelzfixierkomponente umfasst
ein Substrat, und
eine auf dem Substrat angeordnete äußere Schicht, wobei die äußere Schicht aus einer Lösung gebildet ist, die ein Phosphonitriltrimer, Harz und einen Säurekatalysator in einem Lösungsmittel umfasst,
wobei das Phosphonitriltrimer die Struktur aufweist:
wobei Rᵢ und Rᵢᵢ unabhängig voneinander ausgewählte Alkylgruppen oder Derivate davon sind, und
wobei das Phosphonitriltrimer mit dem Harz vernetzt ist.

## Revendications

1. Élément de fixage comprenant :
un substrat ; et
une couche externe disposée sur le substrat, dans lequel la couche externe comprend un trimère phosphonitrilique, dans lequel ladite couche externe est formée à partir d'une solution comprenant un trimère phosphonitrilique, une résine et un catalyseur acide dans un solvant,
dans lequel le trimère phosphonitrilique a la structure :
dans laquelle Rᵢ et Rᵢᵢ sont des groupes alkyle choisis indépendamment ou des dérivés associés, et dans laquelle le trimère phosphonitrilique est réticulé avec la résine.

2. Élément selon la revendication 1, dans lequel la résine comprend des résines thermoplastiques et thermodurcissables, choisies dans le groupe constitué par les polycarbonates, les polyesters, les polyuréthanes, les polystyrènes, les polyaryléthers, les polyarylsulfones, les polysulfones, les polyéthersulfones, les sulfures de polyphénylène, l'acétate de polyvinyle, les polyacrylates, les polyvinyl acétals, les polyamides, les polyimides, les résines amino, les résines phénoliques, les résines phénoxy, les résines époxy, les résines d'oxyde de phénylène, les copolymères de polystyrène et d'acrylonitrile, les copolymères d'acétate de vinyle, les copolymères d'acrylate, les résines alkyde, les copolymères styrène-butadiène, les résines styrène-alkyde, le polyvinylcarbazole, et les mélanges associés, éventuellement dans lequel la résine est choisie dans le groupe constitué par un polyol acrylique, un polyol polyéther, un polyol polyester et les mélanges associés.

3. Élément selon la revendication 1, dans lequel le catalyseur acide est choisi dans le groupe constitué par l'acide p-toluène sulfonique, l'acide dinonylnaphtalène sulfonique, l'acide inonylnaphtalène disulfonique, l'acide dodécylbenzène sulfonique et les mélanges associés.

4. Élément selon la revendication 1, dans lequel le substrat comprend un matériau choisi dans le groupe constitué par les métaux et les polymères.

5. Élément selon la revendication 1, dans lequel le trimère phosphonitrilique est présent en une quantité de 5 à 95 pour cent en poids du poids total de la couche externe, éventuellement
dans lequel le trimère phosphonitrilique est présent en une quantité de 50 à 75 pour cent en poids du poids total de la couche externe.

6. Élément selon la revendication 1, dans lequel la résine est présente en une quantité de 5 à 95 pour cent en poids du poids total de la couche externe.

7. Élément selon la revendication 1, dans lequel le trimère phosphonitrilique a une masse moléculaire (Mm) de 300 à 900 ou
dans lequel la couche externe a une épaisseur de 0,1 à 50 µm.

8. Élément selon la revendication 1 qui est un élément xérographique, éventuellement
dans lequel l'élément xérographique est choisi dans le groupe constitué par l'élément de fixage et l'élément de photorécepteur.

9. Élément selon la revendication 8, dans lequel l'élément de fixage est choisi parmi un élément de pression, un élément de fixage, un élément donneur et un élément de chauffage.

10. Élément selon la revendication 1, dans lequel un rapport du trimère phosphonitrilique à la résine est de 0,5 à 3.

11. Élément selon la revendication 1, dans lequel l'élément a une résistance sensiblement plus élevée à la dégradation thermique par rapport à un élément sans la couche externe.

12. Élément de fixage selon la revendication 1 dans lequel l'élément de fixage est choisi dans le groupe constitué par une bande de pression, un rouleau de fusion, une bande de fixage et un rouleau de pression, comprenant en outre éventuellement d'autres couches choisies dans le groupe constitué par une couche de libération externe, une couche intermédiaire et une couche adhésive.

13. Appareil formant une image pour former des images sur un support d'enregistrement comprenant :
une surface rétentrice de charge pour recevoir une image latente électrostatique dessus ;
un élément de développement pour appliquer du toner sur ladite surface rétentrice de charge pour développer une image latente électrostatique pour former une image développée sur ladite surface rétentrice de charge ;
un élément de film de transfert pour transférer l'image développée de ladite surface rétentrice de charge à un substrat de copie ; et
un élément de fixage pour fixer les images de toner sur une surface dudit substrat de copie, ledit élément de fixage comprenant
un substrat, et
une couche externe disposée sur le substrat dans lequel ladite couche externe est formée à partir d'une solution comprenant un trimère phosphonitrilique, une résine et un catalyseur acide dans un solvant,
dans lequel le trimère phosphonitrilique a la structure :
dans laquelle Rᵢ et Rᵢᵢ sont des groupes alkyle choisis indépendamment ou des dérivés associés, et
dans laquelle le trimère phosphonitrilique est réticulé avec la résine.
